

# UNITED STATES PATENT OFFICE.

WILLIAM T. WHITEHEAD, OF MAGOG, CANADA, ASSIGNOR OF ONE-HALF TO  
HENRY D. DUPEE, OF BOSTON, MASSACHUSETTS.

## ANILINE-BLACK DISCHARGE.

SPECIFICATION forming part of Letters Patent No. 499,691, dated June 13, 1893.

Application filed February 21, 1893. Serial No. 463,250. (No specimen.)

*To all whom it may concern:*

Be it known that I, WILLIAM T. WHITEHEAD, a subject of the Queen of Great Britain, residing at Magog, in the Province of Quebec, 5 Dominion of Canada, have invented an Improvement in Aniline-Black Discharge, of which the following is a specification.

My invention relates to the production of white or colored patterns or figures in cloth 10 by a discharge on an aniline-black ground, and my invention has for its object the method of producing cloth having such patterns or figures, substantially as will be described.

15 I first print, blotch, slop-pad, or dye the cloth until it is thoroughly saturated with a solution of aniline-black produced by aniline oil or salts of aniline according to any of the well known receipes therefor. The cloth is 20 then dried sufficiently to prevent the color from spreading, and I then print the pattern thereon in my improved discharge, in the usual manner. The aniline-black is thereafter developed by passing the cloth through 25 an aniline-aging machine, or by steaming with or without pressure. If desired, the cloth may be soaped, dried and finished in the usual manner. During the process of developing the aniline-black color the portions 30 of the cloth covered by the discharge throw off the black ground color, and the finished cloth presents the pattern clearly and sharply defined, without blurring or clouding. If the pattern is to be white I make the discharge 35 mixture by taking six pounds, more or less, of metallic zinc in a finely divided condition, or a like quantity of a zinc compound, such as the oxide, hydrate or carbonate, to provide zinc which is the essential or active element 40 of the discharge, one-half gallon of water, and one and one-half gallons of starch paste (one pound of starch per gallon). The finely divided metallic zinc, or the zinc compound, and the water are thoroughly mixed, and the 45 starch paste is added to give the requisite thickness for proper printing. This discharge is printed on the cloth in any well known manner, in the desired pattern or figure.

If the pattern or figure is to be colored, a 50 pigment color, coal-tar color, dye-wood or

berry extract is added to the discharge mixture.

The zinc, whether present in its metallic state or as a compound, is the essential or active element of the discharge, and tends to 55 fasten or fix the color, but it may be still further fastened by adding albumen to the mixture in such quantity and proportion as the nature of the particular case demands.

In the use of a pigment color, I use four 60 quarts gum tragacanth solution, (three ounces per gallon), in the foregoing mixture, instead of the starch paste, as a thickener, and after the finely divided zinc, or a zinc compound, and the water have been thoroughly mixed, I 65 add the thickener and the color, the quantity of the latter varying according to the depth of the shade desired and the nature of the pigment itself.

In using ultramarine blue, for instance, I 70 take about six pounds thereof for the mixture hereinbefore described.

The color may be produced from a coal-tar color, as for instance safranine, and I then take about six pounds of finely divided metallic zinc or a zinc compound, one and one-eighth gallons of water, one and one-half pounds of starch, and nine ounces safranine, mix thoroughly and boil.

Any one of the coal-tar colors having the 80 property of fixing itself to the fabric when used in combination with finely divided metallic zinc or a zinc compound, may be employed, such as Bismarek brown, methyl blue, methyl violet, &c.

I have found in my experiments that most of the so-called basic colors will fix properly with metallic zinc as the essential or active element of the discharge, but some of the acid colors, such as soluble blue and violet 85 90 and acid magenta fail to properly fix with the oxide and produce good results.

To produce the color from dyewood or berry extract, I may take, for instance, about six pounds of finely divided metallic zinc, or one 95 of the zinc compounds, and mix it with one and one-half gallons of water, adding thereto three pints Persian berry extract, 48° Twaddie, a sufficient amount of starch to produce a good impression on the cloth, and one pint 100

chrome acetate, mixing all the ingredients well together, and varying the quantity of Persian berry according to the shade desired. Extracts of logwood, sapan, fustic, 5 quercitron, bark, &c., may be used to produce other colors.

The metallic zinc, to obtain the best results, should be very finely divided and ground to an impalpable powder previous to its addition to the hereinbefore described mixture.

In another concurrently pending application, Serial No. 458,581, filed January 16, 1893, I have described and specifically claimed the use of a compound of zinc to supply the zinc 15 which is the essential element of the discharge mixture.

I do not desire to confine myself to the exact quantity of metallic zinc or of the zinc compound to be used, nor to the other ingredients, as the same may be varied without departing from my invention, the gist of which consists in the employment of zinc as the essential or active element in the discharge.

I claim—  
25 1. The herein described process of produc-

ing cloth having patterns on aniline-black grounds, which consists in treating the cloth with a solution of aniline-black color, drying sufficiently to keep the color from running, and printing the pattern thereon in a discharge containing zinc as its essential or active element, before oxidation of the aniline color, substantially as described.

2. The herein described process of producing cloth having colored patterns on aniline-black grounds, which consists in treating the cloth with a solution of aniline-black color, drying sufficiently to keep the color from running, and printing the pattern thereon in a discharge containing zinc as its essential or active element, and a color, before oxidation of the aniline-black color, substantially as described.

In testimony whereof I have signed my name to this specification in the presence of 45 two subscribing witnesses.

WILLIAM T. WHITEHEAD.

Witnesses:

JAS. DOLPHIN,  
HUGH JAMIESON.